

Patented July 5, 1927.

1,634,731

# UNITED STATES PATENT OFFICE.

KARL WERNER, OF DRESDEN, GERMANY.

## PROCESS OF PRODUCING SAND MOLDS FOR MOLDING STONE PATTERN PLATES.

No Drawing.

Application filed January 18, 1925. Serial No. 3,541.

The object of this invention is a process of producing sand molds for molding stone pattern plates. This process differs from the known processes of producing sand molds for molding pattern plates in foundries and other plants in so far as by means of sand molds made after this process stone pattern plates can be produced which do not shrink and which, at the same time, are equal in strength to pattern plates made of metal in the usual manner.

By means of this process molds are produced which are perfectly smooth on their outer surface and which do not show the more or less granular structure of the sand as do the sand molds hitherto in use. The molds, to which the present invention relates, are temporary molds which are used only once.

20 The use of sand molds for casting gypsum, cement, marble cement, caseine masses etc. for the purpose of producing figures, reliefs and pattern plates for foundries etc. is well known but the objects after 25 the known processes showed the same roughness of surface as the sand molds owing to the tendency of sand molds of the known type to deprive the above-mentioned masses of their dissolvent, for example water or 30 magnesium chloride. This tendency resulted in the shrinking or sinking in of the above-mentioned masses, and, at the same time, in a considerable reduction of their hardness, which, on the other hand, did not 35 take place, if the masses were poured into non-porous molds impermeable to liquids, and it is the fundamental idea on which this new process is based to eliminate the roughness of the surface of the sand molds, 40 to make them smooth and impermeable to liquids so that the material poured into these molds is no longer deprived of its dissolvent and remains much harder.

To produce the effect described above the sand is impregnated before being molded. I am aware of the fact that a process is known of impregnating sand before molding by treating it with solid chlorate or a saturated solution of chlorate. The addition of chlorate causes a chemical action and reaction between the salt and the material poured into the mold for the purpose of imparting a hard surface to the models. The present invention, however, does not aim at 55 imparting a hard surface to the models and

the material used in making them but to prevent the models from reproducing that roughness of surface unavoidably connected with the employment of sand molds made after all existing processes and to make 60 them perfectly smooth. As the models are cast in smooth molds they naturally will reveal a smooth surface which requires only very little finishing and which will be an exact reproduction of the outlines of the 65 original.

The technical importance of the invention lies chiefly in the fact that the present process permits the quick reproduction of objects and models by means of a cheap molding material like sand, while the objects thus produced need only very little finishing. Of special importance is the present invention in regard to the production of pattern material in foundries, as the pattern plates made after this process do not shrink and can be quicker and more cheaply made than metal plates. By means of the sand molds, on which the process is based, pattern plates are produced perfectly 70 equal in value to metal plates. The process consists in mixing the sand prior to molding with resins, or vegetable pitches, and by heating the surface of the mold 75 later on. By the process outlined here there is formed on the surface of the sand mold a fine film of glass-like coating, resin, varnish etc. which smoothes the roughness of the sand by covering its pores and rendering it 80 impermeable to the dissolvents of the material to be poured into it.

The aim of the present invention is attained also by first molding the sand and impregnating its surface shortly before use 85 by powdering the sand mold with pulverized resins, or vegetable pitches and by subjecting it to the action of a flame later on, or by merely powdering the sand mold with soot or talc.

Models formed in these molds will also 90 show a smooth surface, and will exactly correspond to the dimensions of their originals, as the methods outlined above will smooth the roughness of the sand and make it impermeable to the dissolvents of the material to be cast.

I claim:

1. The process of producing sand molds for molding stone pattern plates consisting in molding the sand first, impregnating its 105 110

surface shortly before use by powdering it with pulverized resins and slightly heating it, whereupon the liquid modelling mass is poured in.

2. The process of producing sand molds for molding stone pattern plates consisting in molding the sand first, impregnating its

surface shortly before use by powdering it with pulverized vegetable pitches and slightly heating it, whereupon the liquid 10 modelling mass is poured in.

In testimony whereof I have affixed my signature.

KARL WERNER.